

June 6, 1944.

L. C. TIENKEN, JR., ET AL

**2,350,574**

## AMMUNITION

Filed July 2, 1940



INVENTORS  
Louis C. Tienken, Jr.  
Milton B. Vordahl  
BY *John J. Smythe*  
D. Werner Smythe  
ATTORNEYS

## UNITED STATES PATENT OFFICE

2,350,574

## AMMUNITION

Louis C. Tienken, Jr., Old Greenwich, and Milton E. Vordahl, Milford, Conn., assignors to Remington Arms Company, Inc., a corporation of Delaware

Application July 2, 1940, Serial No. 343,542

7 Claims. (Cl. 102—43)

This invention relates to the manufacture of an article composed of rolled strip material, and will be described more particularly relating to a rolled paper base wad for a shot shell. The base wad of a shot shell has the function of filling the space at the closed end of the shotshell tube, and has a hole therethrough to allow the powder igniting charge to effect combustion of the powder contained in the shot shell directly above the base wad. The base wad must form a gas tight seal between the outer circumference thereof and the paper tube, and a seal between the powder space and the metal of the shotshell head. In the firing of shells, pressures of the order of 10,000 pounds per square inch are produced, so it is very important that the seal be complete, as otherwise failures will result. The base wads are usually made from strip paper or similar material. This is wound into a roll and then placed in the end of the shotshell tube. Following this, the metal or similar material head is placed over the end of the shotshell tube and a pressure is exerted upon the interior of the tube axially, so as to tightly compress the rolled paper wad and materially permanently deform the base wad, so that it will be a coherent wad and press close against the shotshell tube and the metal head. It is evident that the wad must be in such a condition after axial deformation that it will remain closely adherent to the tube and will prevent gas leakage by the wad (between the wad and the tube) and will also prevent leakage through the spaces between the rolls of paper. Due to extremely high pressures that are developed, it is also necessary that the paper be in such a condition that it will not fracture and thereby allow the passage of the powder gases through the fracture.

One of the objects of the present invention is to provide a treatment for the base wad so that the paper will be in the proper condition to withstand the firing pressure without fracture, to prevent the passage of gas through the rolls of paper, and prevent the passage of gas by the base wad between the tube and the exterior surface of the wad. This becomes of particular importance with varying types of metal and particularly steel shot-shell heads, because, if the head is expanded unduly by the powder pressure upon firing, it will be very difficult to extract the fired shell from the chamber of the gun.

The invention contemplates other improvements, which will become apparent from the following description.

In the drawing:

Fig. 1 is a fragmentary cross sectional elevation of a shotshell tube with the base wad in place before assembly and deformation of the base wad.

5 Fig. 2 presents a cross sectional elevation of a shot-shell head before assembly on the tube of Fig. 1.

Fig. 3 shows the completed assembly of the parts of Figs. 1 and 2.

10 Fig. 4 is a fragmentary elevational view of the assembled shotshell components of Fig. 3 after the metallic element and base wad have been placed in their final form.

Fig. 5 is a fragmentary elevational schematic 15 view showing in exaggerated form the expansion of the head upon firing.

Fig. 6 is a perspective view of a rolled base wad before being placed into the shotshell tube.

Fig. 7 shows a means of placing a rolled base 20 wad into the shotshell tube, and giving the base wad an additional compression.

Fig. 8 is a diagram showing the relation between extraction and the percent of wax in the wad.

25 Fig. 9 is a diagrammatic sectional view of a base wad showing the directional properties of a formed wad made in accordance with this invention.

Fig. 10 is a cross sectional elevation of a formed 30 wad showing bulging of the head of the shell due to the pressure of the base wad against the head when it is not headed properly.

The invention will be described more particularly as used in the conventional shot shell having a paper tube 20, rolled paper base wad 21 (Fig. 4), metallic head 22, battery cup and primer assembly 23. It is to be understood, of course, that this is merely for purposes of illustration and that changes may be made from the specific 40 form that is shown.

As one means of winding the base wad, placing it within the tube and placing the metallic head thereon, reference may be made to the patent to Hurd, No. 635,972. The present invention has particular usefulness in a shotshell having a steel head or a head of similar metal or material not having the same elastic properties as the conventional brass headed shell. The conventional brass headed shell will expand upon 45 firing and then return to its original position so that it may be extracted with ease from the chamber of the gun.

In the conventional use of a shot shell in a gun, an extractor is employed which has a hook 50 that engages the rim of the shell and withdraws

the shell after firing or upon opening of the breech mechanism in the usual manner, and if the head of the shell has become expanded and remains in this condition, it will prevent the proper extraction of the shell from the chamber of the gun. This failure may be due to excessive pressure necessary to pull the shell from the chamber or from the extractor being pulled through the rim of the shell and leaving the shell in the chamber. It has been found when the conventional base wad is used in a steel shell, for example, that the base wad will fail and the powder gases will bulge the shell and result in hard extraction of the shells from the gun. It has also been found that if the base wad is composed of a soft plastic or similar material that the base wad acts as a fluid transmitting agent and transmits the pressure of the powder gases directly to the metallic head, which will also result in a failure of the head to perform satisfactorily.

The paper tube 20 of Fig. 1 may be formed in any of the usual manners and may have the rolled base wad 24 placed therein by a machine such as that disclosed by Hurd, No. 635,072. The rolled paper base wad 24 has a hole 25 through the center for the powder igniting passage. Fig. 6 is a perspective view of such a rolled base wad before deformation. The paper is rolled upon a spindle passing through the hole 25, and takes the form of a spiral roll. The head 26 of Fig. 2 is placed upon the tube 20, as in Fig. 3, with the lip 27 entering the hole 25 of the base wad. In order to have the base wad perform satisfactorily if it is deformed to the shape shown in Fig. 4, it is necessary that it be treated in such a manner as to prevent the leakage of the gas by and through the base wad. It is to be understood that this treatment may take place before or after the paper has been placed in the rolled form. It is also to be understood that other substances besides paper may be used. In order for the base wad to perform satisfactorily, it must have a certain resilience in the transverse direction so that the pressure of the powder acting upon the base wad will not be able to pass between the tube of the wall 20 and the base wad, and this seal must be maintained even when the metallic head expands outwardly under the pressure of the firing of the shell. In Fig. 5 there is shown a diagrammatic sketch of the expansion of the metallic head and paper tube under firing pressure, such as shown in the dotted lines at 28 and 29. At the same time, during this outward movement of the base wad, there must be no leakage or failure in the layers of paper therein, so as to allow the gas to traverse the base wad in an axial direction. A certain amount of the firing pressure is taken up in the base wad by resilience and is not transmitted directly to the head of the shot shell. As a means of accomplishing this, the shotshell wad or material is impregnated, for example, with paraffin wax, although it is to be understood that other waxes besides paraffin wax may be used and other substances giving the wad or paper the proper characteristics. This impregnation, however, must not be complete, or must not saturate the paper, because if the paper is saturated the wad will act as a complete plastic material and will transmit the powder pressure, as mentioned above, directly to the head, and will cause failure thereof. It has been found that, if, for example, the wad be impregnated with from 2 to 15% 75

of the weight of the complete impregnated wad with a wax, that satisfactory results are obtained. Merely by way of example, the wax saturation point of one paper used was about 28% of the total weight of the impregnated wad. The curve of Fig. 8 shows hardness of extraction plotted against the percent of wax in the base wad. As a measure of extraction, a gauge was used to slip over the neck 30 (Fig. 4) of the head of the shell. It is evident that if the neck will not pass into a gauge of a given size, that it will bind in the chamber of the gun and not allow extraction of the shell. This, of course, is a more rigid test than the extractability of a shell from the gun and gives a more positive indication of the effect of the powder pressure on the head of the shell. It has been determined, for example, that when, by this method, 10 to 15% of the shells fired will not enter this gauge, that hard extraction and unsatisfactory performance will occur. It is to be noticed that there is a very marked drop as the wax percentage is increased up to about 2%, and that up to 15% of wax, approximately, may be used without again obtaining hard extraction. As the percentage of the wax is increased, as explained above, a more plastic action results, causing failure of the shell to perform satisfactorily because of the transmission of the powder pressure to the head.

One means of partially impregnating the wad or paper with wax consists, for example, of dipping the formed wad of Fig. 6 in a shallow bath of wax so that one edge of the rolled paper wad is full of wax up to a point, for example, such as 31 of Fig. 6. Then, by subjecting the roll to heat, the wax will be diffused throughout the body of the wad.

Another method in which the wad may be partially impregnated is by placing the wax in a solvent, dipping the wad entirely into the solution, and then driving off the solvent.

Still another method is that of incorporating a certain amount of waxed paper or wax in the beater when the paper for the wad is manufactured. It is to be understood that these are merely examples of the ways in which the wad can be partially impregnated.

Another factor that affects the performance of the shot shell is the condition of the paper of the base wad when it is impregnated. When an unwaxed dry paper base wad is deformed axially to its final form, there will be but little resilience in an outward direction or a direction that is substantially perpendicular to the axis of the base wad. A wad such as this will not expand upon the firing of the shell, so that as the head expands outwardly there will be leakage of gas between the base wad and the tube of the shell. This is illustrated diagrammatically in Fig. 9. As there will be resilience in a dry wad, such as just described, in the directions indicated by the arrows 32, it is necessary for the satisfactory performance of such a wad in a steel shell to have a resilience in the direction, for example, of the arrow 33, and this is obtained by the partial impregnation of the wad with a wax. If the wad is completely impregnated with wax so that it is plastic, there is no resilience, and the powder pressure is transmitted directly to the head, as discussed previously. If the moisture be reduced in the impregnated paper before it is deformed or headed, the optimum results are obtained, and it has been found to be desirable to reduce this, for example, to less than 1% moisture. If

there is moisture in the paper when it is deformed or headed, the results will not be as good as when there is no moisture. The exact reason for this action is not known, but it is believed that a greater transverse resiliency remains in the wad after deformation of the wad by the heading punch in manufacture. A paper in dry form has a property which may be called "stretch," that is, the amount that it can be pulled before the paper actually breaks apart. In one sample of paper, this was found to be about 1%, and the same paper, when deformed in the wad as shown in Fig. 4, did not perceptibly change in this property. However, if the paper of the wad was partially impregnated with wax before the deformation, it was found that the stretch property of the same paper after it had been deformed to the shape shown in Fig. 4, for example, was noticeably increased and in this same paper was found to be between 2 and 2½%. The exact reason for this is likewise not known.

Another means by which the wad may be given more resiliency in the transverse direction is shown in Fig. 7, wherein the wound wad is shown in dotted lines at 34 before it is placed in the tube 20. The die 35 having an aperture 36 with converging walls 37 is provided. The wad 34 is pressed through this die by a punch or suitable means and into position at 38 in tube 20. It is evident that it is compressed in the passage through the die 35.

For the best performance, it is also necessary that the wad be as tightly compressed as possible in the axial deformation thereof, so as to be completely effective as a seal to the powder gases. If a flat heading tool be used to axially deform the wad, the pressure necessary to produce the proper seal at the circumference of the wad with the paper tube 20 will be such that it will force the base of the head outwardly, such as shown at 39 of Fig. 10. As one means of relieving this pressure adjacent the central hole and to prevent the outward projection of the head, a ring may be used on the punch forming the depression or concentric indentation 40, shown in Fig. 4. The portion of the wad at 41 is thereby slightly relieved and the wad is very tightly compressed between the ring 40 and the outer circumference 42, so as to produce the desired satisfactory results.

The problem that has been solved by the present invention is one that has been very troublesome and has prevented the proper development of many types of shot shell heads and, by the invention disclosed herein, it is possible to produce a shot shell that will perform satisfactorily and will properly extract from a gun.

It is to be understood that the invention is not limited to the details shown, and that the appended claims are to be broadly construed.

What is claimed is:

- 5 1. A shot shell having a steel head and a rolled paper base wad, a substantial portion of said base wad having a partial wax impregnation of about 2-15% of the weight of the impregnated base wad.
- 10 2. In the manufacture of shot shells having a base wad of rolled strip paper, the method comprising partially impregnating substantially all of said strip with a wax to the extent of 2-15% of the weight of the impregnated base wad, and then deforming the base wad axially so as to increase the stretchability of the paper.
- 15 3. In the manufacture of shot shells having a rolled paper base wad, the method comprising the steps of partially impregnating substantially all of the paper with wax to the extent of 2-15% of the weight of the impregnated wad, drying the paper, and then deforming the rolled paper wad.
- 20 4. In the manufacture of shot shells having a rolled strip paper base wad, the method of partially impregnating substantially the entire base wad with wax comprising impregnating a portion of the wad with wax and then diffusing the wax through the wad.
- 25 5. A shot shell having a steel head and a rolled paper base wad, substantially all of said base wad having a partial wax impregnation, said impregnation being not over 15% of the weight of the impregnated wad and sufficient so that the wad has the desired resiliency and gas sealing properties.
- 30 6. In the manufacture of shot shells, having a base wad of rolled strip paper, the method comprising partially impregnating substantially all of said strip to an extent not over 15% of the weight of the impregnated wad and sufficient to give the desired resiliency and gas sealing properties, and then deforming the base wad axially so as to increase the stretchability of the paper.
- 35 7. In the manufacture of shot shells having a rolled paper base wad, the method comprising the steps of removing the moisture from the paper of said base wad, partially impregnating substantially all of the paper of said wad to the extent of 2 to 15% of the weight of the impregnated base wad and deforming the rolled base wad.

LOUIS C. TIENKEN, JR.  
MILTON B. VORDAHL